

# UNITED STATES PATENT OFFICE.

CHARLES H. MYERS, OF PHELPS, NEW YORK.

## PROCESS OF COLORING AND FINISHING PICTURES.

SPECIFICATION forming part of Letters Patent No. 257,051, dated April 25, 1882.

Application filed April 13, 1881. (No specimens.)

*To all whom it may concern:*

Be it known that I, CHARLES H. MYERS, of Phelps, in the county of Ontario, and in the State of New York, have invented certain new and useful Improvements in the Process of Coloring and Finishing Pictures; and I do hereby declare that the following is a full, clear, and exact description thereof, reference being had to the accompanying drawings, and to the letters of reference marked thereon, making a part of this specification.

This invention relates to certain improvements in painting or coloring pictures—such as engravings, lithographs, photographs, and the like—and it is principally designed to provide an improved means for coloring portraits; and it has for its objects to more closely imitate nature, and at less expense than the ordinary oil-paintings.

It is well known that the coloring-matter of the human countenance and other parts of the body does not lie in the cuticle or outer skin, which is semi-transparent, but merely shows through it.

The object of my invention in the production of pictures is to follow nature as closely as possible by rendering the paper upon which a picture is printed or photographed semi-transparent, and applying or painting on the colors at the back, then mounting the picture on a suitable backing, and finally finishing it, when required, upon the surface, as more fully hereinafter specified.

In carrying out my invention I prepare a compound of the following ingredients, in about the proportions named, viz: sugar of lead, one and one-fourth ounce; spirits of turpentine, one quart; Canada balsam, one pound.

The sugar of lead is finely pulverized, and the turpentine is poured upon it, and the mixture allowed to stand for two days. The turpentine is then poured off, and the Canada balsam is added to it and dissolved at a gentle heat, the mixture being frequently stirred during the operation.

The paper on which the picture is produced is saturated with this compound by brushing it on or otherwise, and after it has become dry the paper will be semi-transparent and ready for coloring, which is applied at the back, oil-

colors being preferably used. When the colors have become thoroughly dry the back of the picture is cemented to a backing of card-board, canvas, or other suitable material, and the whole subjected to powerful pressure, by which the picture and backing are securely united. The surface of the picture is then finished by touching it up as required.

I am aware that pictures have been prepared by rendering the paper transparent by means of a suitable varnish and painting on the back thereof, and also that such pictures have been pasted upon a backing of thicker paper; but this I do not claim broadly, my invention consisting, in connection with the above-mentioned steps, of the successive steps following, viz: the backing under great pressure, by means of which the picture becomes a component part of the backing, giving the whole an almost perfect resemblance, and touching or finishing the surface in colors to heighten the whole effect.

The sugar of lead, which is one of the ingredients of my compound, is an essential element thereof, for without it that natural appearance, which is the sole object of my invention, cannot be given to the pictures.

Having thus described my invention, what I claim, and desire to secure by Letters Patent, is—

The process of coloring and finishing pictures, consisting, first, in rendering the paper upon which they are painted or photographed semi-transparent by treating the paper to a compound of the following ingredients: sugar of lead, one and one-fourth ounce; spirits of turpentine, one quart; Canada balsam, one pound; second, applying the color to the back; third, cementing the picture to a suitable backing; fourth, securing it to the backing by great pressure, and, fifth, finishing it on the surface, all in the manner described.

In testimony that I claim the foregoing I have hereunto set my hand this 22d day of March, 1881.

CHARLES H. MYERS.

Witnesses:

J. J. McCARTHY,  
W. M. H. FINCH.